

# UNITED STATES PATENT OFFICE.

HENRY GAULT, OF STRASSBURG, FRANCE, ASSIGNOR OF ONE-HALF TO PHILIP DRINKER, OF BETHLEHEM, PENNSYLVANIA.

## PROCESS OF APPLYING COATED FABRICS TO OBJECTS.

1,394,890.

Specification of Letters Patent.

Patented Oct. 25, 1921.

No Drawing.

Application filed March 13, 1920. Serial No. 365,822.

To all whom it may concern:

Be it known that I, HENRY GAULT, a citizen of the Republic of France, residing at Strassburg, Bas-Rhin, France, have invented a certain new and useful Improvement in Processes of Applying Coated Fabrics to Objects, of which the following is a specification.

My invention relates particularly to a process for covering objects with coated fabrics but relates more especially to a process involving the use of fabrics coated with cellulose esters.

The object of my invention is to provide a process by means of which objects may be covered with coated fabrics, particularly fabrics coated with cellulose esters and especially a fabric covered with cellulose acetate, in order to secure the requisite tautness of the fabric.

Another object of my invention is to cover objects in this way in such a manner as to avoid as far as possible the escape of solvents used with the coating materials utilized for coating the fabrics.

Again, a further object is to cover such objects with the minimum amount of hand labor, as in my process much of the hand labor previously used is done away with.

Another object is to obtain a uniform product by utilizing a fabric provided with even thicknesses of the coating material.

Again, another object of my invention is to facilitate the transportation of the products by enabling the objects and covering materials to be shipped separately and combined upon receipt of the same where the completed object is to be utilized.

Another object is to provide a process of this kind which is especially applicable for covering aeroplanes and parts thereof, as for example the wings, ailerons, fins, rudders, tail pieces, etc.

Further objects of my invention will appear from the detailed description thereof contained hereinafter.

While my invention is capable of being carried out in many different ways for the purpose of illustration I shall describe only certain forms of my invention hereinafter.

For example, in carrying out my invention any part of an aeroplane, as for example a

wing thereof, which is to be covered with the coated fabric may be so covered at the factory where the wing is made, or the wing and the coated fabric may be shipped separately to the point of destination where the coated fabric may be applied thereto. In order to apply the coated fabric to the aeroplane wing, a fabric, such for example as linen, cotton or silk is first thoroughly dried in any suitable manner, after which I apply one coating of a coating composition to the under surface thereof in any suitable manner, but preferably by passing the fabric through an artificial leather coating machine of any desired character and supplied with a suitable coating composition, as for example a cellulose acetate coating composition. A composition suitable for this purpose would be a composition containing,

21% cellulose acetate,  
10% phenol,  
69% ethyl alcohol.

It is to be understood, however, that various different ingredients may be used for this coating composition. Among the principal solvents used in the composition, however, may be mentioned acetone, methyl acetate, ethyl acetate, methyl ethyl ketone, acetone oil, methyl acetone, and the same may contain diluents, such for example as benzene or ethyl alcohol, and that in addition some high boiling solvents may be used such as benzyl alcohol, benzyl benzoate, benzyl, acetate, furfural, eugenol, etc., the purpose of which is to prevent the whitening of the materials remaining after evaporation of the solvents. Furthermore, a plastic such as triphenyl phosphate may be added as well as phenol or cresol, and, if desired, a stabilizer may be introduced such as urea. When this coating has dried on the fabric one or more coatings of the same coating composition are applied in a similar manner to the other side of the fabric. During the application and drying of these layers of coating composition on the two sides of the fabric the solvents may be recovered by evaporation as is usual in the operation of artificial leather coating machines. After the coating materials on the two sides of the fabric have dried completely which will ordinarily be accomplished in 48 hours the

fabric is sewn together so as to fit the aeroplane wing. The fabric is in this condition if it is to be shipped apart from the wing and applied thereto at the point of destination. In order to apply the coated fabric to the aeroplane wing the fabric is now soaked in water for about 24 hours until it is completely saturated. The purpose of this step in the operation is to enable a coated fabric 10 to be applied in such a way as to insure the coated fabric becoming stretched completely taut on the aeroplane wing. This is based upon the principle which I utilize, that fabrics which have been coated with cellulose acetate or other cellulose esters such as a cellulose nitrate when dampened with an appropriate liquid which causes the coating to swell up or dissolve at least in part lose their tautness as they appreciably increase in area 15 under these conditions and that thereafter when they are stretched on an object to be covered and dried the desired tautness will be obtained. Instead of soaking the coated fabric in water I may, instead, substitute for 20 the water a dilute aqueous solution of cellulose acetate high boiling solvents, such for example as one of the following two compositions,

90      95% water.      80% water,  
            5% phenol.      20% acetic acid.

Thereupon the wet coated fabric is stretched in any suitable manner and then stretched over the aeroplane wing in any suitable 35 manner by any suitable mechanical means and fastened on the same in any suitable way, as for example by sewing, the application of adhesives, the use of nails, etc. The fabric on the aeroplane wing is then 40 allowed to dry thoroughly for about 24 hours. This makes the fabric taut on the wing. To the dried fabric on the wing I then apply a moistening or coating of a high boiling solvent mixture, such for example as the following composition.

15% acetone,  
45% tetrachlorethane,  
20% alcohol,  
20% benzene.

50 This may be applied for example by means of an air brush. The purpose of applying this high boiling solvent mixture is to enable the coated composition to work into the fabric in case it has become loosened at any 55 place. The liquid washing or moistening material is then allowed to evaporate until the fabric is dry, whereupon the fabric regains its original tension. Along the edges and ribs of the wing, protecting tapes or strips may be applied and to these tapes there may be applied by hand a coating of the cellulose acetate coating material above referred to. The fabric is then given a coating of a drying oil or a suitable varnish such

for example as boiled linseed oil in order to 65 protect it from the access of moisture. The aeroplane wing is now in finished shape. The other portions of the aeroplane, may, if desired, be covered in a similar manner.

While I have described my invention above 70 in detail, I wish it to be understood that many changes may be made therein without departing from the spirit thereof.

I claim:

1. The process which comprises applying 75 a coating of a cellulose ester to a fabric, drying it, then moistening the fabric, attaching it to an object, drying it, and applying a solvent wash.

2. The process which comprises applying 80 a coating of a cellulose acetate to a fabric, drying it, then moistening the fabric, attaching it to an object, drying it, and applying a solvent wash.

3. The process which comprises applying 85 a coating of cellulose ester to a fabric, drying it, then moistening the fabric, attaching it to a portion of an aeroplane, drying it, and applying a solvent wash.

4. The process which comprises applying 90 a coating of a cellulose ester to a fabric, drying it, then moistening the fabric, attaching it to a wing of an aeroplane, drying it, and applying a solvent wash.

5. The process which comprises applying 95 a coating of a cellulose ester to a fabric, drying it, then moistening the fabric, attaching it to an object, drying it, applying a solvent wash and then applying a moisture resisting layer.

6. The process which comprises applying 100 a coating of a cellulose acetate to a fabric, drying it, then moistening the fabric, attaching it to an object, drying it, applying a solvent wash and then applying a moisture 105 resisting layer.

7. The process which comprises applying a coating of a cellulose ester to a fabric, drying it, then moistening the fabric, attaching it to a portion of an aeroplane, drying it, 110 applying a solvent wash and then applying a moisture resisting layer.

8. The process which comprises applying a coating of a cellulose ester to a fabric, drying it, then moistening the fabric, attaching it to an object, drying it, applying a solvent 115 wash and then applying a moisture resisting layer of an oil.

9. The process which comprises applying a coating of a cellulose ester to a fabric, drying it, then moistening the fabric, attaching it to a portion of an aeroplane, drying it, applying a solvent wash and then applying a moisture 120 resisting layer of an oil.

10. The process which comprises applying 125 a coating of a cellulose acetate to a fabric, drying it, then moistening the fabric, attaching it to a wing of an aeroplane, dry-

ing it, applying a solvent wash and then applying a moisture resisting layer of an oil.

11. The process which comprises applying a coating of cellulose acetate to a fabric, drying it, then moistening the fabric, attaching it to the wing of an aeroplane, drying

the latter, applying a solvent wash, drying, and then applying a moisture resisting layer of an oil.

In testimony that I claim the foregoing, I have hereunto set my hand this 18th day of February, 1920.

HENRY GAULT.